

Aug. 28, 1951

C. B. FRANCIS ET AL

2,565,959

## METHOD OF CASTING METAL CONTINUOUSLY

Filed Oct. 4, 1949

3 Sheets-Sheet 1



### *Inventors:*

CHARLES B. FRANCIS and  
RALPH B. PORTER,  
by: Donald G. Dalton  
their Attorney.

Aug. 28, 1951

C. B. FRANCIS ET AL

2,565,959

METHOD OF CASTING METAL CONTINUOUSLY

Filed Oct. 4, 1949

3 Sheets-Sheet 2



FIG. 8.



*Inventors:*

CHARLES B. FRANCIS and  
RALPH B. PORTER,  
by Donald G. Dalton  
their Attorney.

Aug. 28, 1951

C. B. FRANCIS, ET AL

2,565,959

METHOD OF CASTING METAL CONTINUOUSLY

Filed Oct. 4, 1949

3 Sheets-Sheet 3

FIG. 9.



FIG. 10.



*Inventors:*  
CHARLES B. FRANCIS and  
RALPH B. PORTER,  
by: Donald G. Dalton  
Their Attorney.

## UNITED STATES PATENT OFFICE

2,565,959

METHOD OF CASTING METAL  
CONTINUOUSLYCharles B. Francis, Pittsburgh, and Ralph B.  
Porter, Johnstown, Pa.

Application October 4, 1949, Serial No. 119,532

1 Claim. (Cl. 148—2)

1

This invention relates to the casting of metals, and more particularly to the continuous casting of iron and its alloys, including both carbon and alloy steels, whereby whole heats may be cast directly into semi-finished products of great length, such as slabs, blooms, shaped blooms and billets, heretofore produced by rolling from ingots, and certain sections which it is most difficult or impossible to form by rolling, either because the shape of the article or the hot working characteristics of the alloy itself will not permit the necessary rolling or forging. The invention is an improvement over the practice disclosed in United States Patent No. 2,338,781 granted to Ralph B. Porter on January 11, 1944. This is a continuation-in-part of our copending application Serial No. 840, filed January 7, 1948, and now abandoned.

The chief object of the invention is to simplify and reduce the cost of forming semi-finished iron and steel products, such as slabs, blooms and billets, from which finished products, such as plates, sheets, shapes and bars are rolled. Heretofore, these intermediate products have been formed by casting the liquid steel in molds to form solid ingots, heating the ingots to a temperature suitable for rolling and rolling the ingots first on slabbing or blooming mills. Not only is the equipment used for performing these operations very costly, but the process is wasteful of materials, time and labor since the ingots contain pipes and other defects, making it necessary to scrap 10% to 35% of the steel made, and also because of the fuel consumed in heating the ingots and other materials required to condition them for rolling. Our invention reduces the cost of the apparatus required to a small fraction of the cost of a blooming mill and the labor to less than one-third that employed in present practice. The slabs and blooms, furthermore, are fully formed in the time now required to pour the ingots, and under conditions that avoid pipe, so that the scrap loss is less than 1% for any grade of steel produced.

Further objects are to provide for the making of shapes that cannot be rolled and to improve generally on methods previously proposed for the continuous casting of metals. Other objects will become apparent in the following detailed description of the process of our invention which refers to the accompanying drawings for illustration of a present preferred form of apparatus used therein.

In the drawings:

Figure 11 is a longitudinal vertical section

2

through the center of a preferred form of complete assembly of all parts of the apparatus essential in the casting of such a product as slabs in accordance with our invention;

Figures 2 and 3 are cross-sections taken, respectively, along the lines II—II and III—III of Figure 1;

Figure 4 is a partial section showing a portion of Figure 1 to enlarged scale and a stopping and withdrawing head which travels through a continuous mold at the start of a cast;

Figure 5 is a view similar to Figure 1 showing a portion of a modification;

Figure 6 is a horizontal section taken along the line VI—VI of Figure 5;

Figure 7 is a cross-section taken along the line VII—VII of Figure 5;

Figure 8 is a series of sections or shapes difficult or impossible to roll by the conventional method but which may be continuously cast by our invention;

Figure 9 is a longitudinal vertical section through a portion of the mold preferred for metals such as low-carbon steel having relatively high melting points; and

Figure 10 is a cross-section taken along line X—X of Figure 9.

Referring now in detail to the drawings and, for the present, to Figures 1—4, the apparatus which we prefer to employ in carrying out the invention includes a pouring basin and gate 1, an upwardly flaring or V-shaped riser or skimmer 2 (desirable particularly in the casting of certain steels, particularly high alloy steels) and a port 3. All these parts are in the form of flasks made of cast iron or steel plate formed by bending and welding and are lined with refractory material. To provide a skimmer, or for any other reason, gate 2 may be inclined from the vertical at any angle desired.

A continuous horizontal mold 4 is the initial cooling and forming section of the apparatus and is designed for the continuous casting of slabs. The mold has a cooling jacket 5 provided with connections for circulating water therethrough so that all parts, except the inner faces, are kept below the temperature of boiling water during a casting. The mold comprises two parts, a ribbed inner wall 6 cast in one to three sections longitudinally of a high-silicon, low-carbon alloy of iron, resistant to heat and wear, such as that used for diesel engine blocks; and an outer wall 7 which may be formed of ordinary steel plate by bending and welding parts together. This wall is provided with an expansion joint 7a lo-

## 3

cated at, or near, its midsection, is bolted to the casting at the ends as shown, and may be further secured by stud belts entering the ribs of the casting. These ribs strengthen the casting and direct the flow of the cooling water from the inlet to the outlet of each section.

The finish on the inner faces of the casting is of prime importance. These faces must be flat and as smooth as it is practicable to make them, to decrease sliding friction and avoid such troubles in casting as sticking and bleeding of the form in the mold, particularly at the entering or hot end. The smoothing operations are carried out after the casting has been shaken out and stress-relieved, and depend largely upon the care and means taken to produce a smooth surface in casting.

The water inlets and outlets must be large enough to permit a sufficient flow of water through the mold. To hold the outlet water at a temperature just below boiling requires a feed of 50 lbs. per minute for each square foot of mold cooling surface.

Since the heat conductivity of iron and steel is only  $\frac{1}{3}$  that of copper, attempts have been made to use molds made of copper and its alloys. But copper, as compared with iron alloys, is a soft metal and has a low melting point (1981.4° F.). It bonds or adheres to iron or steel at temperatures below its melting point, furthermore, and experience has taught it is not a satisfactory metal for use for this purpose. Apparently, its high heat conductivity plays a minor part in cooling after a shell is formed between it and the liquid steel.

The apparatus shown includes a final cooling section 8 adjacent the mold 4. It consists of a housing provided with conveyor rolls 9 to receive the partly solidified section as it leaves the mold 4, and a number of high-pressure nozzles 10 arranged to deliver jets of a cooling fluid striking the cast section on all sides as it is moved out of and away from the mold. These jets effect rapid solidification of any metal remaining liquid in the central portion of the cast section by quench cooling the outer shell formed as the section moves through the length of the mold. The number of these sprayes depends upon the thickness and the speed of travel of the section, only one being required for a section 2" thick moving at a rate between 8 and 10 feet per minute. For a section 4 inches thick the total water required per minute by these jets is roughly equal to the weight of steel cast per minute.

A stand of motor-driven rough-surface rolls 11 engage the cooled and solidified portion of the cast section and draw it from the mold at a uniform rate. The traction force necessary, as will be shown later, varies with the volume of the mold and the smoothness of its mold surfaces and increases as the height of the pouring basin above the mold is increased.

A continuous high-temperature furnace 12, represented diagrammatically in the drawing, quickly raises the temperature of the quenched shell to a bright red color, i. e., to a temperature approaching that of the interior of the cast section, to avoid quenching cracks and facilitate subsequent shearing and any further forming operations as desired. The furnace has supporting rollers 12<sup>a</sup> on opposite sides thereof. By regulating the cooling to effect solidification of the shell without excessive cooling of the central portion of the section being formed, this reheating of the outer portion can be effected

## 4

in the same time as the cooling by holding the furnace temperature at around 2400° F.

A motor-driven shear 13 is mounted upon a traveling base 14 to move with the piece while making a cut. A stationary shear can be used, but necessitates shutting off the water sprays and stopping the rolls 9 while making a cut. In that case, it is advisable to cut only a few long lengths during the casting of a heat, and to perform the operation of cutting to shorter lengths on a second shear. Shearing is necessary because of the great length of slab it is possible to obtain from a single heat. For example, a 100-ton heat will give a 4" x 36" slab 400 to 410 ft. long.

In using the apparatus described to perform our method, molten steel is poured from a skimmer ladle 15 into the gate 1 to fill it and port 3 rapidly at the beginning of a cast. As shown in Figure 2, a triangular-shaped refractory diverter 16 is disposed in the diverging riser 2, to divide the stream of hot metal and direct the flow along the walls where thick skulls may otherwise build up, causing the stream to channel through the center.

Figure 4 shows the construction of a preferred form of device used to stop the flow of metal through the mold at the beginning of a cast and to withdraw the section as cast until it is long enough to enter roll stand 11. This stopper or head 17 is composed of a block 18 and bars 19 and 20, fitted neatly together and mounted on channels 21 forming a ram effective to close the mold completely except for a very small V-shaped vent in the top surface of the top bar. The bars and block are held together by three or more loosely-fitted removable pins 22. Bars 19 project beyond the bars 20 and have a number of holes drilled in them to form keys with the first metal cast which solidifies against the head and adjacent to the walls of the mold. These interlocks assure that the shell formed by solidification of the molten metal against the cold mold and stopper surfaces will move with the head as it is withdrawn from the mold. The channels 21 are welded to the outer end of the head and are long enough to provide a ram extending entirely through the mold 4, cooling section 8 and traction rolls 11 as the latter by frictional engagement with the channels, may serve to withdraw the head as fast as steel is fed into the mold. Once the section being cast has thus been started, the operation is continuous until the ladle 15 has been emptied.

Figure 5 is a vertical longitudinal section of a modified continuous mold and cooling section corresponding generally to the construction shown in Figure 1, similar parts being designated by the same numerals, but providing straight-line flow of metal through the mold and the simultaneous casting of four large blooms and one billet. In this form of apparatus the flaring or V-shaped skimmer 2' is connected as a horizontal extension of the port 3 and is lined with dense, hard-burned refractory in the bottom but with porous, bonded, molding sand in the top to permit the escape of gases through small holes provided in the upper side of the flask.

To facilitate the work of smoothing the inner surfaces, the mold 4' of this form of apparatus is built in three sections which are bolted together and is provided with longitudinal partitions of steel plate as shown in Figure 6. To provide cooling for these partitions, they are drilled vertically to form a large number of holes spaced apart along the center line. If preferred, these

partitions may be made thicker and cast with a continuous slot formed with a core along the center line of each section. To prevent the liquid steel from solidifying about the port ends of these partitions, the front ends are shielded by hard-burned refractory brick inserted in the port, as shown at 23 in Figure 6. Since these partitions provide increased cooling for the molten steel, the mold can be made somewhat shorter than a mold designed for the casting of slabs.

Figures 9 and 10 show a portion of a mold generally similar to those illustrated at 4 and 4', which is preferred for the casting of metals having melting points above 2000° F. and particularly for low-carbon steel, which enters the mold at temperatures between 2780° F. and 2850° F.

Each mold section has an inner wall 24 cast from metal similar to that used for diesel engine cylinders, an intermediate wall 25 defining an inner cooling chamber and an outer wall 25<sup>a</sup> forming an outer cooling chamber. Cooling water is supplied through inlet 26 at a pressure of 20 to 30 lbs. to the inner cooling chamber from which it flows as indicated by arrows to the outer chamber from which it is discharged through outlets 27 and 27<sup>a</sup>.

For large sections, that is, when the distance from the inlet 26 of Figure 10 to the openings 28 into the outer chamber is more than about 24 inches and always where this distance exceeds 36 inches, the construction should be modified to provide an inlet and outlets at both the top and the bottom, and the openings 28 between the inner and outer chambers placed at the ends of the mold in locations indicated by the symbols P and P' in Figure 10. For small sections, the outer chamber may be omitted. In any case, the large outer chamber plays a minor part in the cooling, but serves as a temperature equalizer and safety device to condense any steam formed in the inner chamber.

With sufficient pressure in the water main, the flow of water through the cooling chambers is regulated by a valve so that the maximum temperature of the water flowing from the outer chamber is below 200° F. Thus regulated, the rate of flow of water in pounds or gallons per minute depends upon the size of the section and rate of withdrawing steel from the mold. In general, 1 lb. of water solidifies 3 lbs. of steel and, for sections more than 2 inches thick withdrawn at the rate of 1 foot per second, the pounds of cooling water required per second is 25 times the perimeter of the section in feet. Any larger quantity of water may be used.

The advantage of this design over that shown in Figures 1, 3, 5 and 6 is explained as follows:

As the liquid steel enters the cold mold, the rate of heat transfer is at first very rapid because of the great difference in temperature between the liquid steel and the surface of the cold mold with which the liquid is in close contact, and also because of the large amount of heat to be absorbed, which includes the heat of fusion of the steel as well as that necessary to cool the steel to the temperature of the mold. As a consequence, the temperature of the inner surface of the thin mold wall rises very rapidly to a temperature far above that at which water boils, with the result that the opposite water cooled surface becomes covered by a layer of steam, which prevents the water flowing through a cooling chamber with a section as large as that shown in Figures 1, 3 and 4 from making

10  
15  
20  
25  
30  
35  
40  
45  
50  
55

contact with the hot surface—a condition similar to that long known as the spheroidal state. It is necessary, therefore, to prevent the water adjacent the hot surface from assuming the spheroidal state and to remove and condense the layer of steam as rapidly as it is formed—results we accomplish by making the cooling chamber in two parts and decreasing the cross-sectional area of the inner chamber so that the cooling water flows through this chamber at a high velocity. In this way, the friction between the fluid interfaces is increased to a point where the film of steam is removed and condensed as rapidly as it forms, and the temperature of the mold wall at the inner face is prevented from rising much above that of boiling water. Thus, since the mold wall is relatively thin, the rate of heat transfer from the liquid steel to the water becomes very rapid.

Because the port 3 constitutes one of the features of our invention which is novel even to the art of continuous casting, it deserves special mention. We provide means for preheating the end of the port adjacent the metal mold, such as electric-resistance heaters in the form of rods 29 of cemented silicon carbide. For maximum effect two of these bars are inserted, one at the bottom and one at the top as shown in Figure 1, each separated from the mold by 1 to 2 inches of refractory, but when due precautions are taken to avoid delays in withdrawing the cast section as soon as the port is filled with liquid metal, one rod inserted in the bottom, as shown in Figure 5, is sufficient. These rods may be exposed to the liquid steel, as shown in Figure 1, or protected, as shown in Figure 5. If exposed, they can be used but once, but if protected, they may be used to cast several heats. In any case, the rods must be long enough to extend across the port and project through the walls of the flask one to two inches to permit electrical connections to be made, as indicated in Figure 6. By energizing the rods and properly insulating them from metal parts of the apparatus, they may be rapidly heated to any temperature desired up to 2700° F., at which temperature all steels are in a fluid or semi-fluid state. The port 3 is thus heated to a temperature approximating that at which the metal freezes. Instead of electrical-resistance heaters, refractory radiant tubes heated with any combustible gas mixture that will give a high temperature may be used, and in some cases it may be possible to heat this part with molten metal, as by shortening the port and shaping its bottom, as indicated by the dotted line 30 of Figure 1. For general application, however, we prefer to use the rods.

The function of these heating elements is important and is best explained as follows: When liquid steel comes into contact with a cold surface, it starts to solidify, forming a film or shell on the surface, and during the 5 to 10 seconds required to fill the gate and port, this shell may increase to a thickness of  $\frac{1}{4}$ " or more, making it impossible to move the withdrawing head without rupturing the shell. With the heater rods in place, the difficulty is easily overcome, for by turning on the current about an hour before a heat is to be cast, the rods and refractories near them can be heated to a high temperature so that no film or shell will be formed when the liquid steel makes contact with them. Therefore, located as they are, they form a parting line between the shell or metal solidified in the gate and port and that solidified in the mold, making it possible to

withdraw the head 17 and cast section even after the gate and port have been filled for several seconds with metal.

With this description of the various parts of the apparatus and their functions, the principles involved in its construction and precautions to be observed in its operation are briefly discussed in the following paragraphs. With the various parts of the apparatus properly built, assembled and firmly mounted and lined up upon suitable foundations, its operation presents no difficulties when carried out as follows:

After making sure that the traction rolls 11 are in perfect working order, the operator, 1½ to 2 hours before the heat is to be tapped, turns the current on to heat the rods 29, slowly at first, and then more rapidly until they are white hot. This heating is best regulated by means of a thermocouple placed near and above the rods. Unless the exit end of the mold is closed, a draft will be produced causing some of the heat to flow through the gate. This closure may be effected by inserting the withdrawing head 17 for a distance of a foot or so into the exit end of the mold. Finally, just before liquid steel is admitted to the pouring basin, water in large volumes is started flowing through the mold, the current heating the rods 29 is turned off, and the withdrawing head is pushed through the mold to within 2 to 6 inches of the entering end thereof, so that it will not be warmed by heat from the rods. In the meantime, the pouring ladle 15 is heated inside as hot as possible with a gas burner.

By the method of our invention, the metal is tapped from the refining furnace into a teeming ladle, in which the metal is held until its temperature is approaching its liquidus point. From this ladle the metal is preferably teemed, or bottom poured into a basin, from which it flows by gravity through the gate and port into the end of the mold, the port wall or walls being previously heated to a temperature sufficiently high to prevent the liquid metal in contact with them from solidifying, and the entrance to the mold being closed by the withdrawing head just before pouring begins. The liquid metal in contact with the cold face of the withdrawing head is rapidly solidified, so that as soon as the port is full, the withdrawing head, or heads, are drawn back through the mold at a speed adjusted so that the volume displaced by the head is equal to or slightly less than the pouring rate, which is kept as low as practicable and varies somewhat not only for different steels, but also during the pouring of a heat.

By this method the dimensions of the mold, as well as the speed of withdrawal, are adjusted to the minimum pouring rate so that the shell of solidified steel formed in the mold is thick enough and strong enough to permit the section to be withdrawn from the mold. As the rate of solidification, that is, the thickness of shell formed in a given time, is practically the same for all steels, and varies inversely as the square of the time, this factor and the minimum pouring rate determine the cross sectional dimensions of the mold, which is limited as to length to about six feet by other factors. From this maximum, the length of the mold may be reduced according to the thickness of the section, to 4 or 5 feet for a slab two inches thick, for example.

The heat of steel is tapped into a teeming ladle fitted with a one-inch diameter nozzle, the smallest practicable, and held in the ladle 20 to 30 minutes to permit the temperature of the steel

to drop as low as practicable for pouring. The nozzle is opened for 2 or 3 seconds over the spare ladle 15, and the steel collected is quickly poured while the teeming ladle is moved by crane to center the nozzle over the pouring basin, and the stopper is raised. As soon as metal starts rising in the pouring basin, the withdrawing head is started moving slowly backward through the mold at a speed of 8 to 10 feet per minute for slabs 4 inches thick by driving the traction rolls 11. If this speed of travel is not fast enough to balance the teeming rate, the teeming is checked momentarily by closing the nozzle with the stopper, and opening it again before the pouring basin is empty. As the head 17 emerges from the mold 4, the water jets are turned on full, and after the slab has been gripped by the rolls 11, the channels 21, bars 20 and block 18 are detached from the bars 19 embedded in the casting by knocking out the removable pins 22.

Once started, teeming should be as nearly continuous as possible, feeding the metal as fast as it is withdrawn from the mold with the withdrawing head or casting moving at the uniform rate of 6 to 8 feet per minute. No attempt should be made to adjust the speed of withdrawal to the pouring rate. It frequently happens, however, that the pouring rate cannot be controlled with the stopper, as in the case of "stickers" or "running stoppers" due to metal freezing in the nozzle or about the stopper or to defective stoppers. In such event, the steel is allowed to flow into the ladle 15 of Figure 1, which may be tilted to pour over the lip into the pouring basin at any rate desired. By tilting this ladle at the start, pouring from both ladles may proceed simultaneously so that this ladle can be much smaller than the teeming ladle, say ⅓ to ½ the size of the latter.

At the end of the pour, there is no head of liquid metal, so that the last 5 to 6 feet of the cast may be piped and the last 2 or 3 feet, representing the metal contained in the skimmer gate and port may be undersize, since it is insufficient to fill the mold. The pinch rolls may be designed to grip undersize as well as full-size sections, so that practically all of this metal can be withdrawn from the apparatus of the design shown in Figure 5. After each heat has been cast, however, it is necessary to remove, inspect and repair both the gate and the port sections, in preparation for the next cast. The mold itself lasts for many heats, but should be carefully inspected for signs of wear after each heat. Any pitting or deep scoring of the inner surface of any section is cause for its removal and replacement with a section having a smooth inner surface.

The principles governing the design and determining the dimensions of the mold will now be explained. Regarding the dimensions of one embodiment of the molds shown in the drawings, these are preferably six feet in length and 4" x 36", inside dimensions, to cast slabs, blooms and billets 4 inches thick, and slabs 36 inches in width, and blooms and billets of any width desired cast in multiples to give a total width of 32 inches. Other factors besides the desired finished size should be considered in fixing these dimensions as follows:

First, the speed of withdrawal must be adjusted to the minimum pouring rate, which in large-scale operations is about two tons (4000 lbs.) per minute, equivalent to pouring a heat of 100 tons in 50 minutes. The capacity of the mold is 6 cu. ft. and, taking the density of liquid steel to be an average of about 475 lbs., the rate

of travel per minute through the mold must be 1.4 or

$$\left( \frac{4000}{6 \times 475} \right)$$

times the length of the mold, or 8.4 feet per minute, making the time the steel is in the mold approximately 43 seconds. As will be shown later, this is the minimum time required to solidify a shell of sufficient rigidity to permit extraction from the mold. This speed may be increased as the thickness of the cast section is decreased, or decreased as the thickness is increased, if the other dimensions (length and width) remain the same. If the other dimensions are changed along with the thickness, then the speed must be adjusted according to the cubical content of the mold to withdraw the steel as fast as it is poured.

For any mold of a given length, the maximum speed of withdrawal is limited by the maximum rate of solidification of the steel, which can be controlled only to a limited extent, as will be evident from the following descriptive explanation. As the liquid steel enters the mold, the surface in contact with the cold mold wall is almost instantly cooled to the liquidus point at which the steel begins to solidify. Because of the great difference in temperature between the two surfaces, the mold wall absorbs heat from the liquidus surface rapidly, causing complete solidification of a thin film in but a fraction of a second. Since the film thus formed is pressed tightly against the mold wall by internal liquid pressure the rapid transfer of heat continues, so that if the steel is admitted to the mold at a temperature but slightly above its liquidus point, the film first formed rapidly increases in thickness to nearly  $\frac{1}{8}$  inch in 1 second,  $\frac{1}{4}$  inch in 3 to 5 seconds, and  $\frac{1}{2}$  inch in 11 to 15 seconds. As the steel solidifies it contracts, and with a shell  $\frac{1}{2}$  inch thick the upper surface and side walls break contact with the mold, slowing the rate of cooling from these surfaces slightly below the rate from the bottom. The heat which it is necessary to extract, in order to solidify the steel remaining liquid, is about 100 cals. per g. and the rate of heat flow is inversely proportional to the thickness of the shell wall and directly proportional to the difference in temperature between the two surfaces of this wall. By water cooling the mold and making its walls thin, this difference is made much greater than when steel is cast in a heavy metal mold, such as an ingot mold, so that the shell formed on the bottom is about one inch thick within 45 seconds, or by the time it reaches the end of a mold 6 ft. long, when the rate of travel is 8 ft. per minute.

Here all surfaces of the sections are quenched to at most 200° C. by jets of water or other fluid, so that the time, T, in seconds, required to complete solidification may be found from the formula

$$H = kS \left( \frac{t-t'}{e} \right) T$$

in which  $H$ =100 cal. per g., 770 cal. per cc. of steel, or 1540 total,  $k$  is the coefficient of heat conductivity for steel=0.11,  $S$ =1 sq. cm.,  $t$  is the temperature in degrees C. of the liquid steel=1500° C.,  $t'$  is the temperature of the outer surface=200° C., and  $e$ , the mean thickness of wall=4 cm. Substituting these values in the formula gives 43.1 seconds as the time required to complete solidification of the section, during which time the section moves forward about 60

inches. This quick solidification is important since it permits the low fluid pressure forcing metal forward to fill the central voids and prevent piping in a slab 4 inches thick and under, but is not rapid enough to assure complete solidification of a slab 6 inches thick in time to prevent piping entirely.

The fluid pressure within the mold is controlled by the height of the pouring basin above the mold. Assuming that the specific gravity of the liquid steel at pouring temperature is 7.7, as compared with water at 4° C., each foot of head=3.25 lbs. per sq. in. In the apparatus shown in Figures 1 and 5, when the pouring basin is filled with metal, the liquid level stands 4 feet above the bottom of the mold, to give a fluid pressure in the mold of 12 to 13 lbs. per square inch, less a small amount for loss of head in fluid flow through the gate. The pouring basin is made no higher because this pressure is sufficient to feed metal to the mold, and a higher pressure may rupture the shell formed in the mold to produce the surface defect known as bleeding, and also increases the force necessary to withdraw the section from the mold. This force is estimated as follows:

Since the ferrostatic pressure is transmitted in all directions undiminished, except for loss of head due to flow, it acts to push the metal through the mold and also to force the thin shell formed against the mold walls. Assuming that this pressure is exerted until the shell is  $\frac{1}{2}$  inch thick or for a distance of 24 inches, the total outward pressure for a slab 36 inches wide and 4 inches thick is

|                                                                 | Pounds |
|-----------------------------------------------------------------|--------|
| 24" $\times$ 80" $\times$ 6 lbs.                                | 11,520 |
| The weight of the slab in the mold=6 cu. ft. $\times$ 480#      | 2,880  |
| 40 Total pressure                                               | 14,400 |
| Subtract pressure against face=4" $\times$ 36" $\times$ 12 lbs. | 1,728  |
| 45 Total pressure to be balanced                                | 12,672 |

Now, the coefficient of friction of steel on steel varies from 0.15 for very smooth surfaces to 0.30 for finish machined surfaces, so the total force required to withdraw the slab from the mold is  $12,672 \# \times 0.3 = 3,802$  lbs., and the power required=

$$6 \times \frac{60}{45} \times \frac{3802 \text{ lbs.}}{33,000} = 0.91 \text{ horsepower}$$

plus that required to operate other equipment. Because withdrawal is started at the port end of the mold and before more than a few inches of steel is admitted, starting friction is ignored, but in practice the power required to operate the equipment is much more than the extracting force.

If the pouring basin is elevated to 8 ft. instead of 4 ft. above the mold the power required to withdraw the slab is almost doubled.

Again, when the shell formed in the mold is  $\frac{1}{4}$  inch thick, the strength of the solidified section will probably not exceed 400 lbs. per square inch, so that the total force per inch of cross-section the shell can withstand is 100 lbs. This force is exceeded by the force of friction when the ferrostatic head is 11 feet, and raising the pouring basin to this height would result in tearing the shell as fast as it is formed, so that the section may be bleeding as it is withdrawn from the mold. As the detached portions of the shell would remain in contact with the mold, they

would gradually grow thicker until eventually they would block the free movement of metal through the mold in the parts to which they are attached.

As the various limiting factors make it impractical to attempt complete solidification in the mold, we resort to the use of high pressure water jets 10 directed against all surfaces of the section as it is withdrawn from the mold, to effect complete solidification of the central portion in a minimum period of time and before the section reaches the withdrawing rolls 11 which of necessity exert considerable pressure upon at least two surfaces of the section. If the section were passed through these rolls while the central portion is still in a fluid or semi-fluid state, the section would be deformed to a considerable extent, and the central portion would be defective in that it would be characterized by a weak, porous structure, similar to that obtained when an ingot is rolled before the central portion has solidified.

Rapid cooling at this point to effect complete solidification also permits feeding of liquid metal to compensate for the contraction or solidification, and assures a solid section free of pipe or remnants of pipe.

The application of the cold water jets has the effect of chilling or quenching the surface to a temperature well below the critical range, or in the range 300° F. to 700° F., leaving the central portion at a much higher temperature, which will vary according to the thickness from about 800° F. for a slab 2 inches thick to about 1800° F. for a slab 4 inches thick. This treatment, therefore, hardens the surface, particularly of the higher carbon steels, develops stresses in the section, and makes it difficult to cut the section into lengths by either shearing or sawing, the only methods of cutting that are rapid enough for the process. To overcome this difficulty, as well as to improve the quality of the product, we pass the section through a reheating furnace 12 to restore the heat to the surface metal and make the temperature of the section more nearly uniform for cutting into lengths suitable for the next forming operation.

From this description, it will be observed that the method of our invention consists essentially of continuously introducing the molten metal through a preheated refractory port into a metal mold, supported in a horizontal or nearly horizontal position and designed for the rapid abstraction of heat to form a shell of solidified metal conforming to the section desired; continuously withdrawing this shell from the mold and rapidly cooling it by direct application of a fluid cooling medium to complete the solidification of the section progressively toward the exit end of the mold so that the liquid metal, under a low head will flow forward to compensate liquid-to-solid contraction of the metal; and

subsequently applying heat to the quenched or chilled surfaces to restore the temperature of the shell to substantially that of the interior and thus relieve stresses developed in cooling and soften the structure for cutting into lengths desired for the next operation.

Having thus described the apparatus used, recited the principles to be observed and the precautions to be taken in designing and constructing it and explained the method to be followed in the continuous casting of steel, we wish to point out that it may also be applied to the casting of other metals, such as copper and nickel, and that various modifications may be introduced in its design and construction without exceeding the scope of the invention as defined by the following claim.

We claim:

In a method of progressively casting an elongated mass of metal of indefinite length, the steps including preheating to a temperature near the freezing point of the metal, the outlet end of a U-tube gate connected to the entrance end of a horizontal mold open at both ends, thereby preventing formation of a shell of solidified metal adjacent said entrance end of the mold, inserting a closure head into the mold from the other end, pouring molten metal into a basin surmounting the inlet end of said gate above the level of the mold whereby the metal flows into said entrance end and against said head, circulating cooling liquid about the mold thereby causing partial solidification of the metal therein, withdrawing said head and thereby pulling from the mold a continuous mass of metal preliminarily shaped therein, discharging sprays of cooling liquid onto the mass immediately it emerges from the mold, to accelerate freezing of the interior thereof, then passing the mass directly through a continuous furnace thereby reheating it exteriorly and tending to equalize the interior and exterior temperatures thereof and finally shearing said mass into predetermined lengths as it emerges from the furnace.

CHARLES B. FRANCIS.  
RALPH B. PORTER.

#### REFERENCES CITED

50 The following references are of record in the file of this patent:

#### UNITED STATES PATENTS

| Number    | Name     | Date          |
|-----------|----------|---------------|
| 894,410   | Trotz    | July 28, 1908 |
| 944,370   | Monnot   | Dec. 28, 1909 |
| 944,668   | Douteur  | Dec. 28, 1909 |
| 2,058,447 | Hazelett | Oct. 27, 1936 |
| 2,121,280 | Bell     | June 21, 1938 |
| 2,225,373 | Goss     | Dec. 17, 1940 |
| 2,242,350 | Eldred   | May 20, 1941  |